

Dec. 16, 1924.

1,519,508

**G. A. RICHTER**  
INTERRELATED PROCESS OF AND APPARATUS FOR PRODUCING  
SULPHATE AND SULPHITE PULP  
Filed Aug. 18, 1923



*Inventor:*  
George A. Richter.  
by George A. Richter, May 22, 1875.

## UNITED STATES PATENT OFFICE.

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE.

INTERRELATED PROCESS OF AND APPARATUS FOR PRODUCING SULPHATE AND  
SULPHITE PULP.

Application filed August 18, 1923. Serial No. 658,101.

*To all whom it may concern:*

Be it known that I, GEORGE A. RICHTER, a citizen of the United States, residing at Berlin, in the county of Coos and State of New Hampshire, have invented new and useful Improvements in Interrelated Processes of and Apparatus for Producing Sulphate and Sulphite Pulp, of which the following is a specification.

10 In Letters Patent No. 1,427,125, granted on August 29, 1922, I have described a process of producing sulphite pulp by digesting wood chips or other cellulosic material in the presence of an acid liquor consisting of 15 a solution of sodium sulphate and sulphurous acid, and I have also explained that the soda may be recovered and again used. Although the acid solution which is employed therein for digesting the chips has as its 20 base a soluble sulphate, the pulp produced may be referred to as "sulphite" pulp, inasmuch as the fiber liberation occurs in the presence of sulphurous acid.

The object of the present invention is to 25 provide for the simultaneous production of both sulphite and sulphate pulps with a marked economy of operation; to reduce the number of kinds of raw materials which are required for the production of these pulps; 30 to reduce the quantity of lime which is ordinarily utilized for causticization in a sulphate process of digestion to only that amount which is required because of relative differences in the amount of the two pulps; 35 which are produced simultaneously; and to prevent or reduce the accumulation of lime sludge which marks the ordinary commercial production of sulphate pulp.

In carrying out my invention, it is necessary 40 to utilize as raw material only sulphur and caustic soda, the sulphur being utilized for producing  $SO_2$  gas for the acidulation of the cooking liquor in the sulphite side of the system and for making up sulphur losses, 45 and the caustic soda being added to the sulphate side of the system to make up losses of active alkali in the digestion of the pulp and in the recovery of the soda constituents in the smelting furnaces. A part of the sulphur may be also added in the sulphate side of the system to increase the sulphidity of the cooking liquor when required, as set forth in the application, Serial No. 421,769,

filed November 4, 1920 and renewed February 9, 1923, filed by Douglas H. McMurtrie and myself. Theoretically, if the relative pulp productions are in correct proportion, there is no necessity to use lime as a raw material, but inasmuch as in practice it is practically impossible to maintain the relative 55 productions of the two forms of pulp in proper proportion, it is necessary to employ certain amounts of lime for causticizing the raw liquor for use in the sulphate side of the system. I wish at this point to make it 60 clear that for the purpose of utilizing some designating terms for distinguishing the two interrelated processes, I refer to that process in which a soluble sulphate and a soluble sulphite dissolved in an acid solution 65 is employed for the digestion of the pulp as the sulphite process, or sulphite side of the system, in contradistinction to that process in which the wood is digested in the presence of an alkaline solution comprising 70 caustic soda and sodium sulphide, by which "sulphate pulp" so-called is produced. In general, it may be said that in carrying out my interrelated process in 75 which part of the wood chips are digested in an alkaline liquor and the other part of the chips in an acid liquor, the waste liquor from each digester after being concentrated by the evaporation of a part of its aqueous constituent is delivered to a smelting furnace 80 for the recovery of the inorganic content. These two furnaces are preferably so arranged that in one there is maintained an oxidizing atmosphere for the recovery of a part of the soda in the form of sodium carbonate 85 and sodium sulphate, while in the other furnace a reducing atmosphere is maintained for the recovery of the soda in the form of sodium sulphide and sodium carbonate with doubtless some sodium sulphate. The recovered smelt from the first-mentioned furnace is then acidified for use as liquor in the sulphite digester, whereas the smelt from the reducing smelting furnace, after being causticized if necessary, is 90 employed as the alkaline liquor in the sulphate digester. Thus it will be seen that the soda in one form or another passes in a cycle 95 through the sulphate digester and through the sulphite digester and back again. If in 100 the recovery of the soda from the waste 105

- liquor of the sulphate digester it is exposed to a reducing atmosphere for the production of the alkali as sodium sulphide and sodium carbonate, that which is recovered 5 may be used in forming fresh liquor for the same sulphate digester, in which case a part of the waste liquor is diverted before it reaches the smelting furnace and is delivered for admixture with and the neutralization 10 of the waste acid liquor from the sulphite digester, so that its mineral constituents are then recovered together with the mineral constituents of the sulphite waste liquor in the form of sodium carbonate and 15 sodium sulphate, inasmuch as in the smelting furnace last-mentioned an oxidizing atmosphere has been maintained, so that in either case whether the recovery of the mineral constituents of the sulphite waste 20 liquor is accomplished in the presence of an oxidizing or a reducing atmosphere, and the mineral contents of the waste liquor from the sulphite digester is accomplished in the presence of an oxidizing or a reducing 25 atmosphere, a part of the sulphur and the soda is caused to traverse in one form or another throughout the entire system and be utilized in the formation of both the acid and the alkaline cooking liquors.
- 30 On the accompanying drawing I have shown diagrammatically and most conventionally a system for pulp liberation, said system including the various instrumentalities which may be employed in carrying out 35 the interrelated processes embodying my invention. In using the term "system", I mean thereby to include the various mechanical instrumentalities and connections which constitute a means for the practice 40 of the entire process.
- Referring to drawings, 1 indicates what 45 may be termed for convenience the sulphate digester of the system, inasmuch as the pulp produced thereby is commercially termed "sulphate" pulp, although in the digestion of the wood no sulphate, except that which 50 may be adventitiously present, is in the liquor, and if present, forms no function in the digestion. This digester is charged with cellulosic material such as 55 spruce chips and an alkaline cooking liquor, which consists of an aqueous solution of caustic soda and sodium sulphide. After the chips have been cooked in the alkaline liquor at the usual temperatures and pressures for 60 the usual length of time, the contents of the digester are delivered through a pipe or conduit 2 to a blow-pit or receptacle 3. Through a screened outlet indicated at 4 a part of the 65 black liquor may be forced by a pump through a pipe 6 to a tank 7, which for convenience may be termed a tank for undiluted black liquor. From this tank a certain amount of the black liquor may be delivered 70 by a valved pipe 8 to the top of the digester

for the next cook, inasmuch as the liquor contains a certain small quantity of sodium sulphide and caustic soda. From the blow-pit 3 the pulp and the remainder of the black liquor may be forced by a pump 9 through a conduit 10 to any suitable washing machine, by which the pulp is washed and separated from the black liquor. I preferably employ for this purpose a washing machine such as illustrated and described in Letters Patent, No. 1,421,664, dated July 4, 1922, to Brown, Martinson, Moore and Parker. The pulp which is separated during the washing process is transmitted by a conduit 11 to the usual screens 80 (not shown) wherein knots, specks and foreign matter are removed from the pulp so that the latter may be employed for the manufacture of paper. On the drawing, the washing machine is only conventionally illustrated and is indicated at 12. Subsequently I will explain the treatment to which the black liquor is subjected after delivery from the washing machine 12.

At 13 I have indicated a digester for the digestion of cellulosic material in an acid cooking liquor, and to distinguish it, this digester is here referred to as the sulphite digester, inasmuch as the cooking liquor is acid. In this case the cooking liquor consists of an acid solution of a soluble sulphate and preferably a soluble sulphite such as disclosed in my application, Serial No. 661,240 filed September 6, 1923. Preferably this acid liquor comprises about 4% to 7% free  $\text{SO}_2$  and 0.2% to 2% combined  $\text{SO}_2$  as sodium sulphite and 2% to 4% sodium sulphate. In this case it will be noted that the basic metal employed in the formation of the cooking liquor in both digesters is the same, namely sodium, and that sulphur is employed in both liquors, either as  $\text{SO}_2$ , or in combination with sodium as sulphite, sulphate or sulphide. The sodium is combined as caustic soda and sodium sulphide in the alkaline liquor and is combined as sodium sulphate and sodium sulphite in the acid liquor. After the chips have been cooked at a temperature of say  $275^{\circ}$  to  $300^{\circ}$  F. for ten to twelve hours in the digester 13, the contents of the digester are blown through the blow-pipe 14 to a blow-pit indicated at 16. From this blow-pit the waste liquor and the pulp are forced by a pump 17 through a conduit 18 to a storage tank 19, from which they are pumped by a pump 20 through a conduit 21 to a pulp washing machine indicated as a whole at 22. This washing machine is preferably substantially similar to that indicated conventionally at 12. After the separation of the pulp from the waste liquor, it is conducted through a conduit 23 to the usual screens (not shown) prior to the formation of the screened pulp into paper. The pulp produced by the cooking opera- 130

tion in digester No. 1 is herein termed "sulphate" pulp, while that produced from the digested 13 is designated "sulphite" pulp, partly because of the commercial usage of the former term and in order to distinguish the pulp produced in the digester 13 from that pulp commercially known as "sulphate" pulp.

There remains now to be described the means by which the soda is recovered from the waste liquor on the two sides of the system and utilized in both processes of digestion. In each case the waste liquor is concentrated by the evaporation of a portion of its water content in any convenient manner and the residuum is smelted in a smelting furnace for the recovery of the soda in one or another of several compounds. Preferably for the concentration of the waste liquor in each case I employ a multiple-effect evaporator, that for the alkaline waste liquor being indicated conventionally at 24 and that for the acid liquor being indicated at 25. On the drawing it will be observed that there is a conduit 26 for delivering the alkaline waste liquor to the multiple-effect evaporator 24 and a conduit 27 for delivering the acid liquor from the washing machine to the multiple-effect evaporator 25. 28 and 29 indicate two smelting furnaces. Preferably I employ that type of combined smelting and boiler furnace which is illustrated and described in the patent to Moore and Quinn, No. 1,326,414, dated December 30, 1919, in which case the waste liquor is first heated while maintained under external pressure so as to generate therein an explosive force so that when liberated in the combustion chamber of the furnace the waste liquor is disintegrated and the combustible content thereof consumed, and although on the drawings the furnaces are only conventionally indicated, one may, by referring to the Letters Patent last herein referred to, obtain the details of the furnaces which I prefer to employ. There is this difference, however, between the two furnaces which I utilize; namely, that in one case the smelt is subjected to a reducing atmosphere, whereas in the other, the smelt is subjected to an oxidizing atmosphere. In the present instance the furnace in which a reducing atmosphere is maintained is that indicated at 29, in order that a portion of the soda may be recovered in the form of sodium sulphide as well as sodium carbonate, together with some sodium sulphate. The furnace 28, on the other hand, in the present instance is the one in which an oxidizing atmosphere is maintained so that the soda is recovered from the alkaline liquor in the form of sodium carbonate and sodium sulphate. The acid liquor should be neutralized preferably before it is evaporated and burned, and consequently from the dissolving tank 30

into which a part of the smelt from the furnace 28 is delivered for solution in water or any alkaline liquor, the alkaline liquor is forced by a pump 31 through a conduit 32 into the storage tank 19 which receives the pulp and waste liquor from the sulphite digester. A sufficient quantity of this alkaline liquor is mixed with the acid liquor in the storage tank 19 to neutralize it.

The smelt from the reducing smelting furnace 29 is delivered into a dissolving tank 33 containing water so that the sodium compounds which are soluble may be dissolved therein. This solution comprising sodium sulphide, sodium carbonate and some sodium sulphate ordinarily requires to be causticized by the addition of lime and consequently I have illustrated on the drawing at 34 a causticizing tank equipped with an agitator. A sufficient quantity of lime is added for reaction with the sodium carbonate for the production of caustic soda. After the causticizing operation, the liquor is pumped by a pump 35 through a conduit 36 and a filter press 37 to a mixing tank 38, so that there may now be added to the alkaline liquor sufficient caustic soda to make up losses occurring in the original liquor during the digestion and the recovery of the soda. I have indicated conventionally at 39 a tank for containing a caustic soda solution, a portion of the contents of which may be delivered through a valve pipe 40 to the mixing tank 38. From this mixing tank the alkaline liquor may now be pumped by a pump 41 through a pipe 42 to the sulphate digester 1 for the cooking of a fresh batch of chips. Any deficiency in sulphidity may be made up by adding sulphur to the mixing tank from a receptacle 43. Sulphur in any event is added, on the sulphite side of the system, in the form of  $SO_2$  from the sulphur-burner gases, in acidifying the cooking liquor for digester 13.

Returning now to the recovered soda from the oxidizing furnace 28, the greater part of the smelt is delivered to a dissolving tank 44 containing water or an alkaline liquor. This solution which, it will be recalled, contains both sulphate and carbonate of soda is now ready to be acidulated for use in digester 13 for the production of sulphite pulp. Any suitable apparatus may be utilized for acidulating this liquor, so that I have indicated conventionally at 45 a pair of towers 115 through which the alkaline solution may be passed in series and in counter-current flow to  $SO_2$  gas for supplying the solution with sufficient sulphur dioxide to convert the sodium carbonate to sodium sulphate and sodium sulphite and to furnish the solution with the requisite amount of free  $SO_2$ . On the drawing, I have indicated a pump 46 by which the alkaline liquor from the dissolving tank 44 is pumped through a pipe 47 to 120

130

the top of the left-hand tower indicated at 45. Each of these towers is preferably provided with a mass of inert interstitial material such as spiral brick. The liquor after 5 passing through the left-hand tower is pumped by pump 48 through pipe 49 to the top of the right-hand tower, and after emerging from the bottom of the last-mentioned tower is delivered by a conduit 50 to a storage tank 51, from which it may be forced 10 by a pump 52 through pipe 53 to the top of the digester 13 for use in cooking a batch of chips therein. Sulphur burner gas may be delivered to the lower end of the right-hand tower through a gas main 54, and after 15 passing upwardly through the tower is conducted by a conduit 55 to the lower end of the left-hand tower from the top of which the waste gases are vented through an outlet 56. I may reiterate that in describing the conventionally illustrated towers for acidulating the alkaline liquor so that it may be used in the sulphite digester there 20 is no intention on my part to indicate that other forms of apparatus may not be used, as ordinarily I employ acid gas such as relieved from the sulphite digester in effecting a high acidulation of the liquor.

From the foregoing description, it will be 30 apparent that the soda which is dissolved in the acid liquor employed in the production of the sulphite pulp is recovered and utilized in an alkaline liquor for the production of sulphate pulp and, conversely, 35 the soda in the waste alkaline liquor from the sulphite digester is recovered and employed in an acid liquor for the production of sulphite pulp. Consequently, the soda in a soluble form is carried in a complete cycle 40 through the sulphate and sulphite digesters for the digestion of the raw cellulosic materials.

There are many other advantages incident to the process which I have herein described 45 and which will be apparent to those skilled in the art without my attempting to enumerate them. I may advert to the fact, however, that there is a decided advantage in employing as raw materials only caustic soda 50 and sulphur, both of which, as previously stated, may be introduced in the sulphate side of the system herein described. It is true that in practical operation due to the impossibility of maintaining a relative pulp 55 production on both sides of the system, a certain quantity of lime must also be employed for causticizing the soda ash prior to its delivery to the sulphate side of the system, but it is quite apparent that the amount 60 of lime which thus must be employed is much less than that which is ordinarily employed in the usual sulphate process of pulp production. At the risk of repetition, I may call attention to the fact that in the production 65 of sulphite cooking acid liquor for

producing the sulphite pulp, sodium carbonate as delivered from the sulphate side of the system is as suitable for reaction with SO<sub>2</sub> to form sodium sulphite as caustic soda would be, whereas the caustic soda supplied to the liquor for the sulphate digestion replaces that sodium carbonate which is ordinarily used and which requires lime for causticization. The amount of lime saved corresponds to the amount of sodium carbonate delivered from the sulphate side of the system, this amount of sodium carbonate being equivalent to sodium losses in the sulphite side of the system. For example, if in the sulphite side of the system there is 75 lost the equivalent of a certain amount of soda ash per ton of pulp, this is replaced by an equivalent amount of sodium carbonate from the sulphate side of the system, which in turn is compensated for by a sodium constituent in the form of sodium hydroxide, directly supplied to the alkaline cooking liquor so that there is a resulting saving of lime.

On the drawing, which is wholly conventional and diagrammatic, I have made no attempt to indicate the relative dimensions and location of the various instrumentalities or to show the details of the several instrumentalities. For example, I have omitted, as being no part of the present invention, any means for recovering and using the relief from the sulphite digester, or the SO<sub>2</sub> from the blow-pit vapors and gases, or any means for effecting, if desired, the fermentation of the waste liquor on the sulphite side of the system for the formation and recovery of alcohol, all of which are conventionally indicated in my application Serial No. 661,240, filed on September 6, 1923.

I do not herein claim specifically the subject-matter shown, described and claimed in my application Serial No. 661,241, filed on September 6, 1923, in which the soda content of the acid liquor from the sulphite digester is recovered in an oxidizing atmosphere, and in which the soda content of the waste alkaline liquor from the sulphate digester is recovered in a reducing atmosphere. Nor do I herein claim the subject matter claimed in my said application Serial No. 661,240.

What I claim is:—

1. A process of fiber liberation, which 120 comprises digesting raw cellulosic material in an acid cooking liquor containing a soluble sodium compound, digesting raw cellulosic material in an alkaline cooking liquor containing a soluble sodium compound, and recovering sodium compounds from the waste acid cooking liquor resulting from one digestion and using the same 125 in the formation of the alkaline cooking liquor for the other digestion.

2. A process of fiber liberation, which comprises digesting raw cellulosic material in an acid cooking liquor containing a soluble sodium compound, digesting raw cellulosic material in an alkaline cooking liquor containing a soluble sodium compound, and recovering sodium compounds from the waste cooking liquor resulting from one digestion and using the same in the formation of the cooking liquor for the other digestion, and vice versa.

3. A process of fiber liberation, which comprises cooking raw cellulosic materials, one batch in an acid liquor and another batch in an alkaline liquor, and using as the basic compound for the liquor of each batch, those soluble inorganic compounds recovered from the other liquor after the raw material is cooked therewith.

4. A process of fiber liberation, which comprises cooking raw cellulosic material in two batches, one in an acid liquor containing sodium compounds and the other in an alkaline liquor containing sodium compounds, and forming each cooking liquor with sodium compounds recovered from the other liquor after the cooking therewith has been completed.

5. A process of fiber liberation, which comprises recovering sodium compounds from waste alkaline cooking liquor, forming an acid cooking liquor from such compounds and cooking cellulosic material therewith, recovering sodium compounds from the acid waste liquor resulting therefrom, and forming an alkaline cooking liquor from such recovered sodium compounds.

6. A process of fiber liberation, which comprises digesting raw cellulosic materials in successive batches, one in an alkaline cooking liquor and the other in an acid cooking liquor, and forming each liquor with inorganic compounds derived and recovered from the other liquor after the cooking operation therewith.

7. An interrelated process of producing both "sulphate" and "sulphite" pulps from raw cellulosic materials, which comprises using compounds of the same basic metal successively in an alkaline cooking liquor and in an acid cooking liquor, by recovering compounds of said metal from each of such liquors, when spent, and employing such compounds in the formation of the other cooking liquor, and digesting batches of raw cellulosic materials with such acid and alkaline liquors respectively.

8. An interrelated process of manufacturing sulphate and sulphite pulps from raw cellulosic materials, which comprises using compounds of the identical basic metal recovered from the waste cooking liquor employed in producing one of such pulps in forming the cooking liquor for producing the other of such pulps.

9. An interrelated process of manufacturing sulphate and sulphite pulps from raw cellulosic materials, which comprises using compounds of the identical basic metal recovered from the waste cooking liquor employed in producing one of such pulps in forming the cooking liquor for producing the other of such pulps, and making up losses in said basic metal by adding soluble compounds of such metal to one of such liquors.

10. In the manufacture of chemical wood pulp, recovering sodium compounds from the alkaline waste liquor used in producing such pulp, forming a solution thereof, acidifying such solution with sulphur dioxide, and cooking cellulosic material with such acid solution.

11. In the manufacture of chemical wood pulp, cooking cellulosic material in a sulphurous acid solution of a sodium salt, cooking cellulosic material in an alkaline solution of another sodium compound, neutralizing the waste acid cooking liquor with the waste alkaline cooking liquor, recovering sodium compounds from the resulting liquor in an alkaline solution, and cooking cellulosic material therewith.

12. In the manufacture of chemical wood pulp, a cyclic process comprising cooking cellulosic material with an acid solution of sodium-sulphur compounds recovered from the waste hereinafter-mentioned alkaline cooking liquor, and cooking cellulosic material with an alkaline solution of sodium-sulphur compounds recovered from the waste first mentioned acid cooking liquor.

13. In the manufacture of chemical wood pulp, a cyclic process comprising cooking cellulosic material with an acid solution of sodium-sulphur compounds recovered from the waste hereinafter-mentioned alkaline cooking liquor, cooking cellulosic material with an alkaline solution of sodium-sulphur compounds recovered from the waste said acid cooking liquor, and making up losses in sodium during such cyclic operation by adding soluble sodium compounds to the alkaline cooking liquor.

14. A process as herein described, comprising cooking raw cellulosic material in a sulphurous acid solution of sodium sulphate and sodium sulphite, neutralizing the waste acid cooking liquor, smelting the sodium compounds of said waste liquor in a reducing atmosphere and recovering the resulting sodium compounds in an alkaline solution, causticizing the said solution with lime and removing the resulting insoluble carbonate therefrom, and cooking cellulosic material in the final alkaline solution.

15. A process as herein described, comprising cooking raw cellulosic material in an alkaline solution of caustic soda and sodium sulphide, smelting the sodium com-

5 pounds of the waste cooking liquor in an oxidizing atmosphere and recovering the resulting sodium compounds in solution, acidifying such solution with sulphur dioxide, and cooking cellulosic material in such acid solution.

- 10 16. A process as herein described, comprising cooking raw cellulosic material in an alkaline solution of caustic soda and sodium sulphide, smelting the sodium compounds of the waste cooking alkaline liquor in an oxidizing atmosphere and recovering the resulting sodium compounds in solution, acidifying such solution with sulphur dioxide, cooking cellulosic material in such acid solution; smelting the sodium compounds of the waste acid cooking liquor and recovering the resulting sodium compounds in an alkaline solution, causticizing any sodium carbonate in said solution with lime and removing the resulting insoluble carbonate, and cooking raw cellulosic material in the resulting solution, thereby completing a cyclic operation.
- 15 17. A process as herein described, comprising cooking raw cellulosic material in an alkaline solution of caustic soda and sodium sulphide, smelting the sodium compounds of the waste alkaline cooking liquor in an oxidizing atmosphere and recovering the resulting sodium compounds in solution, acidifying such solution with sulphur dioxide, cooking cellulosic material in such acid solution, smelting the sodium com- 30 pounds of the waste acid cooking liquor
- 35

and recovering the resulting sodium compounds in an alkaline solution, causticizing any sodium carbonate in said solution with lime and removing the resulting insoluble carbonate, adding caustic soda to said alkaline solution to make up losses in sodium occasioned by the said operations, and cooking cellulosic material with the resulting liquor, thereby completing a cyclic operation. 40

18. A process as herein described, comprising cooking raw cellulosic material in an alkaline solution of caustic soda and sodium sulphide, smelting the sodium compounds of the waste alkaline cooking liquor in an oxidizing atmosphere and recovering the resulting sodium compounds in solution, acidifying such solution with sulphur dioxide, cooking cellulosic material in such acid solution, smelting the sodium compounds of the waste acid cooking liquor and recovering the resulting sodium compounds in an alkaline solution, causticizing any sodium carbonate in said solution with lime and removing the resulting insoluble carbonate, adding caustic soda to said alkaline solution and such sulphur as may be needed to secure the desired strength in caustic alkalinity and sulphidity and cooking cellulosic material with the resulting alkaline liquor. 45 50 55

In testimony whereof I have affixed my signature.

GEORGE A. RICHTER.